

## UNITED STATES PATENT OFFICE.

WILLIAM H. GRIMDITCH, OF PHILADELPHIA, PENNSYLVANIA, ASSIGNOR TO PHILADELPHIA STORAGE BATTERY COMPANY, OF PHILADELPHIA, PENNSYLVANIA, A CORPORATION OF PENNSYLVANIA.

## WOOD SEPARATOR AND METHOD OF PREPARING SAME.

No Drawing.

Application filed March 5, 1923. Serial No. 623,066.

One object of this invention is to provide a novel succession of steps for the preparation of a dry, porous, wood separator for use in electric batteries, and the invention especially contemplates a method of drying separators which have been subjected to a wet, porosity-giving treatment, without the warping and splitting which heretofore has made impractical the use of such separators.

10 I further desire to provide a wood separator particularly adapted for use in a dry charged battery and which, while being free from objectionable matter and relatively porous, shall be practically water-free and 15 without tendency to warp or split.

In carrying out my invention, I make sheet separators of Douglas fir, Port Orford cedar, cypress, or any other suitable wood, with or 20 without ribs, suitably cut with an allowance for shrinkage across the grain, although, in ordinary sizes, they may be cut to the desired finished length along the grain either before or after the treatment and drying.

The separators, individually or in convenient lengths, are first subjected to a wet treatment to remove resinous or other matter and increase their porosity; as for instance, they may be boiled in water or subjected to 25 a treatment in a solution of caustic soda or other suitable solvent.

After treatment, the wet separators are placed in a suitable dryer, supported between gratings of expanded metal, wire netting or metal rods, or between ordinary battery plate grids. If made of iron, the supporting structures should be lead-coated or 30 tinned to prevent rust, or they may be made of Monel or similar non-rusting metal. The grating may be of any suitable construction 35 which will allow currents of air from the fans of the dryer to enter between and act uniformly on the separators and which will 40 at the same time provide sufficient mechanical support to overcome the tendency of the 45 separators to warp on drying.

The dryer is preferably equipped with humidity and temperature controlling means so that currents of air of predetermined

humidity and temperature may be supplied to the separators. The drying is carried on 50 preferably at a temperature in the neighborhood of 200° F., and during the early part of the drying treatment the relative humidity of the incoming air is run up to approximately 90% following a short initial period 55 at comparatively low humidity for the rapid removal of surface water. As the drying proceeds, the humidity is gradually reduced until practically all the free water has been removed from the separators, at which point, 60 practically dry air may be used to remove the last traces of free water.

Under these conditions, the drying out of the separators proceeds slowly and the shrinkage takes place evenly so that the tendency of the wood to warp or curl is greatly reduced. Ordinarily, from one to three 65 days will be required to dry wet treated separators by the above described method; but the time may be longer or shorter depending on the type and design of separator, the means for support, and the treating and drying conditions, as well as upon other factors.

Wood separators prepared by the above 75 described method come out of the dryer flat and will remain flat in stock until used. They are relatively porous as compared with similar separators of dry raw wood and at the same time possess good insulating 80 properties and ample mechanical strength for use between the plates of storage batteries.

I claim:

1. The method of preparing wood separators, which comprises treating them in a solution adapted to increase their porosity, and thereafter drying the separators by subjecting them to the action of air currents of progressively decreasing humidity. 85

2. The method which comprises the subjection of wet wood separators to the action of warm air of progressively decreasing humidity. 90

3. The method of drying wet wood separators which comprises subjecting them to 95

relatively humid air currents and thereafter subjecting them to progressively drier air currents.

4. The method of drying wet wood separators which comprises forcibly holding them so as to prevent warping and subjecting them to the action of air currents of progressively decreasing humidity.

5. The method of drying wet wood separators which comprises supporting said separators between gratings and subjecting them to the action of a current of warm air of initially high and progressively decreasing humidity.

WILLIAM H. GRIMDITCH.